

## MANUFACTURE OF VISCOSE RAYON

August Brötz, Kurt Richter, Wilhelm Wachtendorf, and Kurt Heuer, all of Erlenbach (Main), Germany, assignors to American Enka Corporation, Enka, N.C., a corporation of Delaware

No Drawing. Filed Feb. 18, 1957, Ser. No. 640,617

Claims priority, application Germany Feb. 20, 1956

4 Claims. (Cl. 18—54)

This invention relates to the production of regenerated cellulose articles such as fibers, films and the like from viscose. More particularly this invention relates to the production of said articles having substantially all skin area, high strength and high fatigue resistance.

A need for a very high tenacity viscose rayon yarn exists in the industry today in order to compete with other synthetic fibers. In recent times, research has been directed toward ever increasing the strength and improving other physical properties of viscose rayon suitable for tire cord or other industrial cords requiring high tenacity and long flex life.

It is known that a definite relationship exists between the strength of rayon yarn and the skin structure of the yarn. Rayons of the high tenacity type have a comparatively thick skin in contrast to the older types of textile rayons which have a very thin skin. As a general rule, the strength of the yarn increases as the percentage of skin area increases and the percentage of core decreases. Furthermore, it is known that yarns having a large degree of skin have a lower swelling value as compared to yarn of little or no skin.

The skin and core as referred to herein are not different types of material but occur from the same stream of viscose. However, it has been established that the orientation and crystallinity of the cellulose molecule in the skin area are different from that of the core area. Generally in the art, the skin portion and core portion of rayon fiber are distinguished by differences in dyeing characteristics between the two portions. A method for determining the skin and core areas of viscose in which the difference in dye absorption is used to differentiate skin from core is set forth in U.S. Patent No 2,536,014.

The formation of a yarn having a considerable degree of skin area may be influenced in different ways. For example, viscose rayon yarns which have a relatively thick skin may be produced by regenerating the cellulose in the presence of a viscose additive which modifies the regeneration-coagulation process of the viscose in the acid spinbath.

Among the viscose modifiers known today are those compounds disclosed in British Patent No. 741,728, U.S. Patents Nos. 2,535,044, 2,535,045, 2,536,014 and 2,696,423. A large number of other such additives are also in the literature.

Although in some instances these viscose modifiers exert a favorable and pronounced influence upon the physical properties of the yarn produced in their presence, however, from an operational point of view it is not very desirable to use modifiers in the process for the production of viscose rayon. Great difficulty is usually encountered when viscose modifiers are used.

In the first place, it is exceedingly difficult to control the amount of additive, especially in the spinbath. If the additive is permitted to build up in the spinbath, the effect of the additive in many cases notably decreases; and in some cases, an inferior yarn will be produced.

The undesirable buildup may occur from the fact that the effect of the modifier is dependent upon being incorporated in the viscose. Also, certain additives are decomposed by the acid and accordingly present difficult removal and spinning problems. Furthermore, the spinbath in the viscose process is constantly being spent in operation and must be regenerated by adding fresh sulphuric acid and removing the excess sodium sulphate. Regeneration of spinbath containing these additives present many operational problems. Thus, it would be desirable to operate without the additives.

Also, by varying the spinning constants a yarn of varying degrees of skin thickness may be produced. By varying the acid concentration the skin thickness can be increased by either increasing or decreasing the acid concentration depending upon other spinning constants. It is known that in general increasing the salt content of the spinbath, as well as lowering the temperature of the spinbath, influences the production of yarn with increased skin thickness. Also, the viscose may be varied to influence skin formation such as increasing or decreasing the sodium hydroxide content, decreasing the aging of the viscose, increasing the amount of  $CS_2$  used during xanthation and increasing the cellulose content thereof.

It is interesting to note that the various factors are interrelated but their effects are not necessarily additive.

Although the general idea of varying the coagulation-regeneration process conditions to produce viscose rayon yarn with some skin is old, the problem of selecting the optimum spinning conditions is by no means simple. Up to the present it was considered that a yarn having over 50% skin could not be produced without sacrificing other yarn properties unless a viscose modifier is employed. Furthermore, unmodified skin filaments heretofore produced have peripheries which are highly crenulated.

Also, in the art today it is known that by varying the spinning conditions and without spinning in the influence of a modifier, yarns which have a dry strength of only slightly more than 3 grams per denier can be produced. In view of the present demand for high strength yarn, these strength values are very inadequate. However, when the known optimum spinning conditions are employed, it is necessary to take undesirable steps in the production of the the yarn, for example, the use of high  $CS_2$  concentrations in the xanthation.

A very high strength yarn may be produced by the so-called Lilienfeld process in which viscose is extruded into a coagulating bath containing sulphuric acid generally in the amount of 60-70% by weight. The spinning or coagulation bath treatment may be followed by a secondary bath also having a relatively high sulphuric acid content. However, other physical properties are not improved and, in most instances, are poorer. The yarn produced by the Lilienfeld process is very brittle and is almost worthless for use in articles which require good extensibility and good fatigue resistance.

While the above-mentioned known methods for producing a yarn having high strength and a high degree of skin represent valuable advances in the art, further improvements in the yarn properties without at the same time presenting spinning problems are needed.

Therefore, it is an object of the present invention to provide a process for producing a regenerated cellulose yarn from viscose having substantially all skin and other improved properties without spinning in the presence of a viscose modifier.

The above and other objects will become apparent from the following more complete description of the instant invention.

In accordance with the present invention, viscose having sodium hydroxide in the amount of 6% or less by weight and a maturity of about 40-46 gamma number is spun into a coagulating spinbath containing about 17-19% sodium sulphate, 4.5-6.0% sulphuric acid, and zinc sulphate, the concentration of which is dependent upon the concentration of the sulphuric acid. It is preferred that the ratio of the acid content to the zinc sulphate content be 1.2-0.8 to 1. After a short travel through the spinbath, the freshly spun yarn is directed into a second hot weakly acid bath where the yarn is stretched in the conventional manner to an extent of at least 85%.

Yarns produced according to this process have dry strength values of 430-450 g./100 denier and corresponding high wet strength values of 270-300 g./100 denier. The elongation values of the yarn are 8-12% in the dry state and 24-26% when wet. Also, the swelling values are in the region of only 70%. The most remarkable fact is that the cross-section of the yarns reveals filaments which have at least 80% skin and which have peripheries of notably reduced crenulation. Also, the yarns have enhanced abrasion and fatigue resistance values.

It is important to the present invention that the percentage of sodium hydroxide in the viscose be not more than 6%. There appears to be no defined lower value for the percent caustic. Generally, it is preferred that the alkali content be no lower than 4.5. However, a viscose with even a lower alkali may be used. In any case, the sodium hydroxide should be sufficiently high to render the viscose amenable to the conventional filtering and spinning processes. The maturity of the viscose is not critical in the present invention. But it is preferred that the viscose be aged to a ripeness of about 40-46 gamma number.

Also, it is important that the concentration of materials in the spinbath be maintained between certain defined ranges. It is necessary that the sulphuric acid be kept at 4.5-6.0%. Above 6.0% the skin thickness of the yarn notably decreases, below 4.0% many spinning problems arise. The concentration of salts in the spinbath should be maintained at certain levels in order to retain their skin formation effect. For example, the optimum concentration of sodium sulphate in the present invention is 17-19%. The concentration of zinc sulphate is varied depending upon the amount of acid in the spinbath. It has been established that the optimum concentration of the zinc salt is reached when the ratio of acid to zinc salts is 1.2-0.8 to 1. In other words, when the acid level is 4.5% the smallest concentration of zinc sulphate should be about 3.8%; and when the acid level is 6.0% the largest concentration of zinc sulphate should be about 7.5%.

Although low acid spinning is known, comparatively slight variations in the composition of the viscose or in the composition of the spinbath was thought to prevent satisfactory spinning. This is clearly evidenced by the fact that in commercially useful processes, the art has found it imperative to stay within narrow limits with respect to the cellulose and alkali contents of the viscose and the constituents of the spinbath, with ordinary commercial spinning employing at least 7.0% sulphuric acid.

It has now been recognized that a commercially useful viscose rayon process may be employed at relatively low concentrations of acid when the viscose composition and the composition of the sulphuric acid coagulating bath are so balanced to permit the production of regenerated cellulose filaments having improved tenacity, flexibility and characterized by an exceptionally high degree of skin.

The process may be more fully illustrated by reference to the following examples which are not to be construed as limiting the present invention in any respect.

#### Example I

Alkali cellulose prepared from cotton linters and aged

to give a viscose solution viscosity of 50-60 poises was xanthated in the usual manner with 37% CS<sub>2</sub>. The xanthate thus obtained was dissolved with caustic soda solution to provide a viscose which contained 7.3% cellulose and 5.5% NaOH. After aging to a maturity of 42 gamma number, deaerating and filtering, the viscose was extruded in a spinbath which contained 4.9% H<sub>2</sub>SO<sub>4</sub>, 17.1% Na<sub>2</sub>SO<sub>4</sub> and 5.0% ZNSO<sub>4</sub>. The coagulating bath had a temperature of 62° C. and the spinneret employed was of the conventional type and had 720 orifices, each orifice having a diameter of 60 microns.

The freshly spun yarn was directed through the spinbath for a distance of 17 cm. and out of this first bath into a second bath. In this second bath which contained 2% H<sub>2</sub>SO<sub>4</sub> and had a temperature of 90° C., the yarn was given a stretch of 90%. The drawoff speed of the yarn was 60 meters per minute. Later the yarn was aftertreated in the usual manner, such as washing, desulphurizing, drying, etc. However, before finally drying the yarn was given an additional stretch of 3-10%. The dried thread was given a twist of 120 turns per meter.

The physical properties of 1650 denier yarn produced in the above manner were as follows. In the dry state the strength of the yarn was 435 g./100 denier and the elongation was 7.8%. In the conditioned state the strength of the yarn was 291 g./100 denier and the elongation was 24.4%. The swelling value of the yarn was 70.9%.

#### Example II

In order to illustrate the critical balance of the spinning variables and to show how the yarn properties are affected thereby, experiments were run using conditions other than the preferred conditions of the present invention. In this respect it was found that the desirable yarn properties of the present invention were not obtainable. Also, the skin area of the yarn was considerably less.

For example, viscose prepared in identical manner as in Example I was extruded into a spinbath containing 6.5% H<sub>2</sub>SO<sub>4</sub>, 17.5% Na<sub>2</sub>SO<sub>4</sub> and 3.5% ZNSO<sub>4</sub>. Other spinning conditions and aftertreating of the thread was the same as described in Example I. The physical properties of yarn produced were 350 g./100 denier dry strength, 10.0% dry elongation, 210 g./100 denier wet strength and 22.0% wet elongation.

What is claimed is:

1. A process for the production of regenerated cellulose articles having substantially all skin from viscose comprising spinning a solution consisting essentially of viscose containing sodium hydroxide in the amount of less 6% by weight into a coagulating spinbath consisting essentially of 17-19% sodium sulphate, 4.5-6.0% sulphuric acid, and zinc sulphate, directing the spun article out of said spinbath into a second bath containing dilute sulphuric acid, and stretching the spun article in the second bath to an extent of at least 85%, the concentration of zinc sulphate being adjusted so that the ratio of sulphuric acid in said spinbath to zinc sulphate is 1.2-0.8 to 1.
2. A process for the production of regenerated cellulose articles having substantially all skin from viscose comprising spinning a solution consisting essentially of viscose containing 4.5-6.0% by weight of sodium hydroxide into a coagulating spinbath consisting essentially of 17-19% sodium sulphate, 4.5-6.0% sulphuric acid, and zinc sulphate, directing the spun article out of said spinbath into a second bath containing dilute sulphuric acid, and stretching the spun article in the second bath to an extent of at least 85%, the concentration of zinc sulphate being adjusted so that the ratio of sulphuric acid in said spinbath to zinc sulphate is 1.2-0.8 to 1.
3. The process as defined in claim 2 wherein the viscose is spun at a maturity of 40-46 gamma number.
4. A process for the production of viscose yarn having at least 80% skin comprising spinning a solution consisting essentially of viscose containing 4.5-6.0% by

weight of sodium hydroxide into a coagulating spinbath consisting essentially of 17-19% sodium sulphate, 4.5-6.0% sulphuric acid, and zinc sulphate, directing the spun yarn out of said spinbath into a second bath containing about 2% sulphuric acid and having a temperature of about 90° C. and stretching the yarn in the second bath at least 85%, the concentration of zinc sulphate being adjusted so that the ratio of sulphuric acid in said spinbath to zinc sulphate is 1.2-0.8 to 1.

## References Cited in the file of this patent

## UNITED STATES PATENTS

2,535,044 Cox ----- Dec. 26, 1950  
2,535,045 Cox ----- Dec. 26, 1950

## FOREIGN PATENTS

204,280 Australia ----- Mar. 8, 1956

UNITED STATES PATENT OFFICE  
CERTIFICATE OF CORRECTION

Patent No. 2,947,597

August 2, 1960

August Brötz et al.

It is hereby certified that error appears in the printed specification of the above numbered patent requiring correction and that the said Letters Patent should read as corrected below.

Column 4, line 50, for "less 6%" read -- less than 6% --.

Signed and sealed this 31st day of January 1961.

(SEAL)

Attest:

KARL H. AXLINE  
Attesting Officer

ROBERT C. WATSON  
Commissioner of Patents